

# United States Patent

Bass

[15] 3,647,439

[45] Mar. 7, 1972

[54] **PHOTOGRAPHIC ELEMENT,  
COMPOSITION AND PROCESS**

[72] Inventor: **Jon Dolf Bass, Rochester, N.Y.**  
[73] Assignee: **Eastman Kodak Company, Rochester, N.Y.**  
[22] Filed: **Oct. 1, 1968**  
[21] Appl. No.: **764,330**

[52] **U.S. Cl.** ..... 96/29 R, 96/48 PD, 96/61 R,  
96/76 R, 96/95, 96/114.6  
[51] **Int. Cl.** ..... G03c 5/54, G03c 5/24, G03c 5/38  
[58] **Field of Search** ..... 96/48 PD, 95, 61, 114.6, 76,  
96/29 R

[56] **References Cited**

UNITED STATES PATENTS

|           |         |               |                  |
|-----------|---------|---------------|------------------|
| 2,084,420 | 6/1937  | Weyde         | ..... 96/114.6 X |
| 3,155,516 | 11/1964 | Blake         | ..... 96/61 X    |
| 3,155,518 | 11/1964 | Blake         | ..... 96/61 X    |
| 3,155,519 | 11/1964 | Blake         | ..... 96/114.6 X |
| 3,330,663 | 7/1967  | Weyde et al.  | ..... 96/114.6 X |
| 3,368,899 | 2/1968  | Blake et al.  | ..... 96/95 X    |
| 3,446,619 | 5/1969  | Gilman et al. | ..... 96/63      |

FOREIGN PATENTS OR APPLICATIONS

|           |        |               |             |
|-----------|--------|---------------|-------------|
| 920,277   | 3/1963 | Great Britain | ..... 96/48 |
| 936,609   | 9/1963 | Great Britain | ..... 96/48 |
| 1,125,646 | 8/1968 | Great Britain | ..... 96/48 |
| 1,453,635 | 8/1966 | France        | ..... 96/48 |

OTHER PUBLICATIONS

Van Veelan et al., *Photographische Korr Espondenz*, Vol. 99,  
No. 9 pps. 139-145, Sept., 1963

*Primary Examiner*—Murray Katz

*Assistant Examiner*—Harry J. Gwinnett

*Attorney*—W. H. J. Kline, R. E. Knapp and B. D. Wiese

[57] **ABSTRACT**

Photographic elements, compositions and processes employing certain stable sources of metal for physical development, including certain metal-organic complexes, such as metal-thiazoline thione or metal-thiazolidine thione complexes or metal-alkyne complexes, provide good images. Silver-dye complexes are especially suitable as a photosensitive material for use with these metal-organic complexes, typically silver-organic complexes.

23 Claims, No Drawings

## PHOTOGRAPHIC ELEMENT, COMPOSITION AND PROCESS

## BACKGROUND OF THE INVENTION

## 1. Field of the Invention

This invention is directed to photographic elements, compositions and processes employing physical development in obtaining a desired image. In one of its aspects, it relates to photographic elements, compositions and processes employing certain stable sources of metal for physical development including certain metal-organic complexes, especially certain silver-organic complexes. In another of its aspects, it relates to photographic elements, compositions and processes employing a silver-dye complex which has the property of forming active sites for physical development upon exposure to radiation in combination with the described silver-organic complexes as stable sources of silver for physical development.

## 2. Description of the Prior Art

Radiation-sensitive coatings based on silver, especially photographic silver halides, and physical development of such coatings, are well known, as described, for example, in Mees, *The Theory of the Photographic Process*, Third Edition, (1966) and British Patent 936,609 issued Sept. 11, 1963. Spectral sensitization of photographic silver halides by addition thereto of a sensitizing dye is also well known. Further, a reaction product, identified as a silver-dye complex of a dye and a water-soluble silver salt, e.g., silver nitrate, which complex is photosensitive is described in French Patent 1,453,635 issued Aug. 16, 1966. A photographic silver halide emulsion which is mixed with such a silver-dye complex has its spectral sensitivity extended into the region of the absorption of the dye. Such silver-dye complexes can be a photosensitive medium in the absence of silver halide, so that energy absorbed by the dye upon exposure is used directly to form sites for physical development. This is disclosed, for example, in French Patent 1,453,635 issued Aug. 16, 1966.

However, the sources of metal, especially silver, for such physical development have not been entirely satisfactory. In many cases they have either been too unstable, releasing the metal at an undesired time, or caused undesired fog and stain. For example, while a silver-thiosulfate complex can be employed as a source of silver for physical development of an image in a photosensitive coating containing a silver-dye complex as the photosensitive material, as described, for example, in French Patent 1,453,635, a silver-thiosulfate complex can produce undesired fog and produce other undesired effects. A silver complex of 4,5-(2,3-D-fructopyrano)-2-oxazolidinethione also has these disadvantages. Accordingly, while sources of silver have been employed for physical development in the described photographic systems, they have not produced desired results in many cases.

Further, there has been a need for sources of silver for physical development which provide desired concentrations of silver ion in particular photographic systems, especially systems employing a silver-dye complex as a photographic component, i.e., desired pAg levels, while providing desired sensitometric properties.

It is accordingly an object of the present invention to provide a photographic element, composition and process, employing an improved stable source of metal, especially silver, for physical development providing desired sensitometric properties.

Another object is to provide a photographic element containing a silver-dye complex capable of forming sites for physical development upon exposure to radiation and containing an improved stable source of metal, especially silver, for physical development of such sites, which is a stable metal-organic complex providing desired sensitometric properties.

Another object is to provide a photographic process for physical development of a latent image in a radiation sensitive metal salt employing an improved stable source of metal for the described physical development.

A further object is to provide a photographic composition, such as a photographic emulsion or developer composition, containing an improved stable source of metal for physical development as described.

5 Additional objects and advantages will be apparent from the following description and claims.

## SUMMARY OF THE INVENTION

- 10 According to the invention improved elements, especially photographic elements, processes and compositions are provided which are suitable for physical development, especially photographic elements, processes and compositions employing a photographic silver-dye complex and are resistant to undesired fog and/or stain by employing an improved stable source of metal for physical development which is a stable metal-organic complex of (a) a metal suitable for physical development with (b) a compound which is:
- a. a thioamide, including
- i. A thiazoline thione and/or thiazolidine thione,
  - ii. A thiopyrimidine,
  - iii. An oxazolidine-2-thione,
  - iv. A dithiocarbamate, and/or
  - v. A thiourea derivative, and/or
- 15 b. a guanyl compound, including
- i. A pseudothiohydantoin,
  - ii. An imidazolidine,
  - iii. An imidazoline, and/or
  - iv. An isothiourea derivative, and/or
- 20 c. a mercapto acid, including
- i. A mercaptocarboxylic acid, and/or
  - ii. A mercaptooxetyl amide, and/or
- 25 d. an alkyne compound, and/or
- 30 e. a hydroxyalkyl carboxylic acid and/or a hydroxy heterocyclic carboxylic acid, and/or
- 35 f. a thiaalkyl compound, including a dithiaalkyl and/or oligothiaalkyl compound, and/or
- 40 g. oxalic acid, a phylene dioxy dialkyl carboxylic acid, and/or succinic acid, and/or
- 45 h. a polymer containing a ligand atom having the property of complexing a metal suitable for physical development including
- i. Polymers wherein the described ligand atom is sulfur, such as
  - 1. Polymers containing thiaalkyl acrylamide units and/or methacrylamide units, and/or
  - 2. Polymers containing thiaalkyl acrylate units and/or methacrylate units.

50 Also, a stable complex of silver with the described polymers according to the invention can provide other desired properties, such as eliminating part of the binder in a photographic emulsion.

## 55 DESCRIPTION OF THE PREFERRED EMBODIMENTS

The described metal-organic complexes are especially advantageous in photographic elements, processes and compositions wherein the metal for physical development is silver and the described stable metal-organic complex is a stable silver-organic complex.

The described stable metal-organic complexes can be employed in a wide range of elements, especially photographic elements, processes and compositions. They can be employed in any photographic element, process or composition where it is desirable to employ a stable metal complex as a stable source of metal, especially silver, for physical development. Various types of photographic elements, processes and compositions, where it is desirable to have a stable source of metal for physical development, are known.

These are described, for example in Mees, *The Theory of the Photographic Process*, Third Edition (1966), pages 324-331, in British Patent 936,609 issued Sept. 11, 1963 and in French Patent 1,453,635 issued Aug. 16, 1966. The described metal-organic complexes are especially suitable in a photographic

element, process and/or composition employing, as a radiation sensitive component, a silver-dye complex which has the property of forming active sites for physical development upon exposure to radiation, as described in French Patent 1,453,635 issued Aug. 16, 1966. The following dyes are representative merocyanine dyes which can be used to form the described radiation sensitive silver-dye complexes:

- a. 3-carboxymethyl-5-[(3-methyl-2-thiazolidinylidene)-ethylidene]rhodanine 420-560 m $\mu$ ;
- b. 5-[(3-methyl-2-thiazolidinylidene)ethylidene]rhodanine 460-570 m $\mu$ ;
- c. 5-[(3-methyl-2-thiazolidinylidene)ethylidene]-2-thio-2,4-oxazolinedione 400-560 m $\mu$ ;
- d. 3-ethyl-5-[(3-methyl-2-thiazolidinylidene)ethylidene]-2-thio-2,4-oxazolinedione 430-540 m $\mu$ ;
- e. 1-methyl-5-[(3-methyl-2-thiazolidinylidene)ethylidene]-2-thiobarbituric acid 430-530 m $\mu$ ;
- f. 3-carboxymethyl-5-[(3-ethyl-2-benzoxazolinylidene)-ethylidene]rhodanine 420-580 m $\mu$ ;
- g. 5-(3-ethyl-2-benzoxazolinylidene) 370-460 m $\mu$ ;
- h. 5-[(3-ethyl-2-benzoxazolinylidene)ethylidene]rhodanine 520-560 m $\mu$ ;
- i. 3-ethyl-5-[(3-ethyl-2-benzoxazolinylidene)ethylidene]-1-phenyl-2-thiohydantoin 520-560 m $\mu$ ; and
- j. 1-carboxymethyl-5-[(3-ethyl-2-benzoxazolinylidene)-ethylidene]-3-phenyl-2-thiohydantoin 520-560 m $\mu$ .

Various dyes, other than merocyanine dyes can be employed as the dye moiety in the described silver-dye complex, including known silver halide sensitizing dyes, such as cyanines, oxonols, hemicyanines, styryls, hemioxonols, benzylidenes, and the like, examples of which are set out in the described Mees reference, pages 198-232.

These silver-dye complexes can be prepared typically by mixing the dyes with a water-soluble silver salt, such as silver nitrate, in a suitable solvent, e.g., water, or can be prepared in a radiation sensitive coating composition in situ without separation or recovery of the silver-dye complex from the coating composition, such as by mixing the desired components in the coating composition before application to a support using techniques well known in the photographic art.

One embodiment of the invention is an element, especially a photographic element comprising a photographic component which is the main photographic component of the desired element and a stable source of metal for physical development, especially a stable source of silver, which is a stable metal-organic complex, preferably a silver-organic complex as described.

An especially useful embodiment is a photographic element comprising a support having thereon a radiation-sensitive silver-dye complex, as described, which has the property of forming active sites for physical development upon exposure to radiation, and a stable source of metal for physical development which is a stable metal-organic complex as described.

The described stable source of metal for physical development according to the invention can be in any location in and/or on the photographic element and/or in a processing composition which provides the desired physical development activity without undesired fog and stain. It can be, for example, in a radiation-sensitive coating and/or an overcoat and/or a coating between the support and a radiation-sensitive coating or some other coating or combination of coatings. It can be in one or more coatings of a receiver sheet employed in a diffusion transfer process and/or in a photographic element and/or processing composition employed in a diffusion transfer process.

While silver is a preferred metal moiety of the described stable metal-organic complexes employed in the invention, other metals which are useful in physical development can be employed. Metals which are members of the electromotive scale below hydrogen are those most commonly employed for this purpose, such as copper, mercury, palladium, platinum, gold, silver, and the like.

A stable source of metal for physical development which is a stable metal-organic complex of (a) a metal suitable for physical development with (b) a thioamide according to the invention is represented by the following formula:

5

(I)



10

15

20

25

30

35

40

45

50

55

60

65

75



wherein M is a metal suitable for physical development, such as silver, copper, mercury, palladium, platinum, gold, and the like; R<sub>1</sub> and R<sub>2</sub> are the same or different and each is hydrogen, alkyl, alkylene, acyl, or aryl; R<sub>3</sub> is alkyl, —S—R<sub>4</sub>, or —O—R<sub>4</sub>, or



any two R groups can, but need not, be joined to form a heterocyclic ring as represented by the broken lines in structure I.

Alkyl suitably contains one to about 20 carbon atoms, typically one to five carbon atoms, such as methyl, ethyl, propyl, butyl, pentyl, decyl and eicosyl. Alkylene suitably contains one to about five carbon atoms, such as methylene, ethylene, propylene, butylene and pentylene. Acyl can be:

Aryl suitably contains six to about 30 carbon atoms, such as phenyl, tolyl, xylol and naphthyl. The described alkyl, alkylene, acyl and aryl can contain various substituent groups which do not adversely affect the stability and availability of metal for physical development of the described complexes and compounds. Suitable substituent groups include for example, carboxyl, hydroxyl and sulfonic acid groups. Such groups can provide advantages in cases in which it is desirable that the described compound have increased solubility in aqueous compositions and/or increased compatibility with, for example, a binder, if one is used.

Examples of silver-thioamide complexes within Formula I which are stable sources of silver for physical development are silver complexes of the following compounds:

- 2-thiobarbituric acid,
- 1,3-diethyl-2-thiobarbituric acid,
- 2-thiouracil,
- imidazolidine-2-thione,
- 1,3-bis(4-carboxyphenyl)-1,3-dimethylthiourea,
- 1,3-bis(2-carboxyethyl)-benzimidazole-2-thione, and
- 4-carboxybenzyl dimethyl dithiocarbamate:



5-carboxy-2-phenyl-4-thiopyrimidine:

5



5-carbethoxy-1-methyl-2-phenyl-4-thiopyrimidine:



5-methyloxazolidine-2-thione:



1-(3,5-dicarboxyphenyl)-5-mercaptopotetrazole

A stable source of metal for physical development which is a stable metal-organic complex of a metal suitable for physical development with a thiiazoline-thione or a thiazolidine thione is represented by the structure:

(II)



wherein R<sub>6</sub> represents atoms completing a heterocyclic ring, such as



or



, wherein R<sub>8</sub> and R<sub>9</sub> are the same or different, and each is hydrogen, alkyl; especially alkyl containing one to five carbon atoms, such as methyl, ethyl, propyl, butyl and pentyl; aryl, as described; carboxyl; hydroxyl; sulfonic acid; and mercapto; R<sub>7</sub> is hydrogen, alkyl, as described, typically alkyl containing one to five carbon atoms, aryl, especially containing six to 20 carbon atoms, carboxyl or sulfonic acid, as described. These are especially suitable sources of silver for physical development according to the invention.

Examples of suitable silver thiazoline thione complexes which are stable sources of silver for physical development are stable silver complexes of the following compounds:

- 3-carboxymethyl-4-methyl-thiazoline-2-thione, 3-(2-carboxyethyl)-4-methyl-thiazoline-2-thione,
- 3-(3-carboxypropyl)-4-methyl-thiazoline-2-thione,
- 3-(4-carboxybutyl)-4-methyl-thiazoline-2-thione,
- 3-(5-carboxypentyl)-4-methyl-thiazoline-2-thione,
- 3-carboxymethyl-4-methyl-5-carboxy-thiazoline-2-thione,
- 3-(2-carboxyethyl)-4-methyl-5-carboxy-thiazoline-2-thione,
- 3-(3-carboxypropyl)-4-methyl-5-carboxy-thiazoline-2-thione,
- 3-carboxymethyl-4-methyl-5-carbethoxy-thiazoline-2-thione,

6

3-(2-carboxyethyl)-4-methyl-5-carbethoxy-thiazoline-2-thione,

3-(3-carboxypropyl)-4-methyl-5-carbethoxy-thiazoline-2-thione,

- 5 3-carboxymethyl-4-carboxymethyl-thiazoline-2-thione,
- 3-(3-carboxypropyl)-4-carboxymethyl-thiazoline-2-thione,
- 3-carboxymethyl-4-methyl-5-acetyl-thiazoline-2-thione,
- 3-(2-carboxyethyl)-4-methyl-5-acetyl-thiazoline-2-thione,
- 3-sulfoethyl-4-methyl-thiazoline-2-thione,

10 3-(m-carboxyphenyl)-4-methyl-thiazoline-2-thione,

3-(1-carboxyethyl)-4-carboxy-thiazoline-2-thione,

3-(1-carboxyethyl)-4-carbethoxy-thiazoline-2-thione,

3-(1-carboxyethyl)-4-(carbethoxymethyl)-thiazoline-2-thione,

15 3-(2-carboxyethyl)-4-(carbethoxymethyl)-thiazoline-2-thione,

3-(2-carboxyethyl)-4-(n-butylsulfonylmethyl)-thiazoline-2-thione,

3-(1,2-dicarboxyethyl)-4-methyl-thiazoline-2-thione, or

4-carboxy-thiazoline-2-thione.

Examples of suitable silver-thiazolidine thione complexes which are stable sources of silver for physical development according to the invention are silver complexes of thiazolidine thione compounds corresponding to the described thiazoline thione compounds. For instance, suitable silver-thiazolidine thione complexes include silver complexes of:

3-carboxymethyl-thiazolidine-2-thione, and

3-carboxyethyl-thiazolidine-2-thione.

A stable source of metal for physical development which is 30 a stable metal-organic complex of a metal suitable for physical development with a thiopyrimidine is represented by the formula:

(III)



40

wherein M is as described; R<sub>10</sub> and R'' are individually hydrogen, alkyl or aryl as described, especially phenyl; R<sub>11</sub> is 45 hydrogen, carboxy, alkyl or aryl, as described.

Examples of suitable silver-thiopyrimidine complexes which are stable sources of silver for physical development are stable silver complexes of:

5-carboxy-2-phenyl-4-thiopyrimidine, and

5-carbethoxy-1-methyl-2-phenyl-thiopyrimidine.

A stable source of metal for physical development which is 55 a stable metal-organic complex of a metal suitable for physical development with an oxazolidine-2-thione is represented by the formula:

(IV)



60

65 wherein M, R<sub>5</sub>, R<sub>6</sub> and R<sub>7</sub> are as described.

Examples of suitable silver-oxazolidine-2-thione complexes which are stable sources of silver for physical development are:

70 5-methyloxazolidine-2-thione,

5-carbethoxoxazolidine-2-thione.

A stable source of metal for physical development which is 75 a stable metal-organic complex of a metal suitable for physical development with a dithiocarbamate is represented by the formula:

(V)



wherein M, R<sub>1</sub> and R<sub>2</sub> are as described; and R<sub>12</sub> is alkyl, aryl, as described, or carboxyaryl, or carboxalkyl, e.g., containing six to 20 carbon atoms, such as carboxybenzyl, carboxyxylyl or carboxyphenyl.

Examples of suitable silver-dithiocarbamate complexes 10 which are stable sources of silver for physical development are stable silver complexes of:

4-carboxybenzyl-dimethyl dithiocarbamate

4-carboxyphenyl-dimethyl dithiocarbamate.

A further stable source of metal for physical development is 15 a stable metal-organic complex of a metal suitable for physical development with a thiourea derivative represented by the formula:

(VI)



wherein M, R<sub>1</sub>, R<sub>2</sub>, R<sub>4</sub> and R<sub>5</sub> are as described; and R<sub>2</sub> and R<sub>5</sub> can, but need not, be joined to form a heterocyclic ring, represented by the broken line in Structure VI. R<sub>2</sub> and R<sub>5</sub> when joined to form a heterocyclic ring can be, for example,



or



wherein R<sub>1</sub> and R<sub>2</sub> are as described.

Examples of suitable stable sources of silver for physical development are complexes of silver with:

2-thiouracil,

thiobarbituric acid,

imidazolidine-2-thione,

1,3-diethyl-2-thiobarbituric acid,

1,3-bis(2-carboxyphenyl)-1,3-dimethylthiourea.

A stable source of metal for physical development which is 50 a stable metal-organic complex of a metal suitable for physical development with a guanyl-containing compound is represented by the formula:

(VII)



wherein M, R<sub>1</sub>, R<sub>2</sub> and R<sub>3</sub> are as described; R is hydrogen, alkyl or alkylene as described; and any two of the described R groups can be, but need not be, joined to form a heterocyclic ring.

An example of a stable metal-organic complex of a metal suitable for physical development within structure VII is a stable metal-organic complex of a metal suitable for physical development with a pseudothiohydantoin represented by the formula:

(VIII)



wherein M is as described, especially silver.

A further source of metal for physical development is a stable metal-organic complex of a metal suitable for physical development with an imidazolidine, especially a 2-thioimidazolidine represented by the formula:

(IX)



wherein M, R<sub>1</sub>, and R<sub>2</sub> are as described; R' is hydrogen or atoms completing a hydrocarbon ring, e.g., alkylene containing four to eight carbon atoms completing a benzene or naphthylene ring, and their corresponding tautomers.

Examples of suitable stable silver-imidazolidine complexes as stable sources of silver for physical development are complexes of silver with:

imidazolidine-2-thione, or

1,3-bis(2-carboxyethyl)-benzimidazole-2-thione.

A source of metal for physical development is a stable metal-organic complex of a metal suitable for physical development with an imidazoline, especially a 2-thioimidazoline represented by the formula:

(X)



wherein M, R<sub>1</sub>, R<sub>2</sub> and R' are as described, and their corresponding tautomers.

Examples of suitable stable silver-imidazoline complexes as stable sources of silver for physical development are complexes of silver with:

2(2-carboxyethylthio)- $\Delta^2$ -imidazoline

2(2-carboxypropylthio)- $\Delta^2$ -imidazoline.

A further source of metal for physical development is a stable metal-organic complex of a metal suitable for physical development with an isothiourea derivative represented by the formula:

(XI)



wherein R<sub>1</sub> and M are as described, with the exception that R<sub>1</sub> is not hydrogen, R, typically being carboxyalkyl or sulfoalkyl. This formula does not include thiourea.

Examples of suitable stable silver-isothiourea derivative complexes as stable sources of silver for physical development 65 are complexes of silver with:

S-(carboxymethyl)isothiourea

S-(2-carboxyethyl)isothiourea

S-(3-carboxypropyl)isothiourea

S-(2-carboxyisopropyl)isothiourea

S-(3-sulfopropyl)isothiourea.

A stable source of metal for physical development is a stable metal-organic complex of a metal suitable for physical development with a mercapto acid, especially a mercapto carboxylic acid represented by the formula:

(XII) [HS-R''-COOH] M

wherein M is as described and R'' is alkylene, such as alkylene containing one to 20 carbon atoms, typically alkylene containing one to five carbon atoms, such as methylene, ethylene, propylene, butylene, pentylene, decylene and eicosylene. R'' can contain substituent groups which do not adversely affect developing action of the described compounds such as alkyl, e.g., alkyl containing one to 20 carbon atoms, typically alkyl containing one to five carbon atoms as described, carboxy, sulfonic acid, mercapto and amino.

Examples of stable silver mercapto acid complexes which are stable sources of silver for physical development according to the invention are silver complexes of:

mercaptoacetic acid,  
mercaptopropionic acid,  
mercaptoisobutyric acid,  
mercaptosuccinic acid,  
alpha-mercaptoadipic acid, and  
L-cysteine.

A stable source of metal for physical development is a stable metal-organic complex of a metal suitable for physical development with a mercaptoacetyl amide represented by the formula:



wherein M and R'' are as described; R<sub>13</sub> and R<sub>14</sub> are the same or different and each selected from hydrogen; lower alkyl, as described; mercapto; carboxyl; sulfonic acid; hydroxyl and phenyl; at least one of R<sub>13</sub> and R<sub>14</sub> being phenyl. The phenyl group can contain various substituent groups which do not adversely affect the stability and availability of metal for physical development, such as carboxyl, hydroxyl, sulfonic acid, and the like.

Examples of silver-mercaptoacetanilide complexes which are stable sources of silver for physical development include silver complexes of:

mercaptoacetanilide,  
mercaptomethylacetanilide, and  
mercapto aceto-p-toluidide.

A metal-alkyne complex which is a stable source of metal for physical development according to the invention is represented by the formula:



wherein M is a metal suitable for physical development, as described; R<sub>15</sub> is hydrogen, aryl, as described, alkyl, as described, or alkylene, also as described, forming a ring with R<sub>16</sub>, as represented by the broken lines in Structure XIV; R<sub>16</sub> is hydrogen, aryl, alkyl, as described, or alkylene, also as described, forming a ring with R<sub>15</sub>; R<sub>15</sub> and R<sub>16</sub> together may represent a keto oxygen; R<sub>17</sub> is —O—R<sub>18</sub>, —S—R<sub>19</sub>,



or an alkylene oxide polymer adduct represented by the formula:



wherein n is an integer, such as an integer from 1 to about 100 or more; R<sub>18</sub>, R<sub>19</sub>, R<sub>20</sub> and R<sub>21</sub> are the same or different and each selected from hydrogen, acyl or alkyl, as described, typically alkyl containing one to five carbon atoms.

Examples of silver-alkyne complexes suitable according to the invention are silver complexes of:

3-methyl-1-butyn-3-ol  
ethylene oxide adduct of 3-methyl-1-butyn-3-ol



3-methyl-1-pentyn-3-ol  
ethylene oxide adduct of 3-methyl-1-pentyn-3-ol



1-hexyn-3-ol  
1-ethynylcyclopentanol



1-ethynylcyclohexanol



ethylene oxide adduct of 1-ethynyl-cyclohexanol



2-propynyl cyclohexylcarboxylate



4-t-butyl-1-ethynylcyclohexanol

3-(diethylamino)-1-butyne



methyl propiolate



3,5-dimethyl-1-hexyn-3-ol

4-(1-hydroxy-2-propynyl)cyclohexene



3-cyclopropyl-1-butyne-3-ol



75 3-phenyl-1-propyn-3-ol





5,5'-thiodisalicylic acid



4-(1,2-dicarboxyethylthio)-5phenylcatechol



S-(o-carboxyphenyl)thioglycolic acid



4-(methylthio)phenol



phenylthioacetic acid



4-(carboxymethylthio)aniline



3-thiavaleric acid

CH<sub>3</sub>CH<sub>2</sub>SCH<sub>2</sub>COOH  
2-(2-furylthio)benzoic acid

(2-furylthio)acetic acid



2(2-furylthio)propionic acid

3-(2-furylthio)propionic acid

(2-furylthio)succinic acid

An especially useful stable source of metal for physical development is a stable metal-organic complex of a metal suitable for physical development with a polymer containing a ligand atom having the property of forming a complex with the described metal.

The described polymer includes any polymer which provides the desired complex, does not cause undesired fog or stain and releases the described metal for physical development. These include homopolymers and copolymers, which include interpolymers of various monomeric and polymeric units. These can contain one or more of the same ligand atom or different ligand atoms.

Any ligand atom is suitable which provides the desired complex. Ligand atoms are described in the book, "Organic Complexing Reagents" by D. D. Perrin, Interscience Publishers, Division of Wiley and Co., 1964, especially the first three chapters.

Suitable polymers containing ligand atoms are described, for example, in the book "Vinyl and Related Polymers" by C. D. Shildknecht, John Wiley and Sons, 1952. Especially suitable polymers are those which provide the advantage of serving as a stable source of silver for physical development as well as serving as a binder to partially or totally replace other binders, such as gelatin, which are used in coatings for photographic elements.

Properties of the desired polymers can vary over wide ranges depending on other components of the photographic element with which they can be used, processing conditions, desired image, and the like, which can be determined by those skilled in the art. For example, average molecular weight and viscosity can vary, but are typically sufficiently high that the desired polymer is solid when in the form of a coating, e.g., about 1,000 to 1,000,000 or more.

A suitable stable metal-organic complex of a metal suitable for physical development with a polymer containing a ligand atom is a metal-organic complex of a metal suitable for physical development, especially silver, with a polymer containing thiaalkylacrylamide units and/or thiaalkylmethacrylamide units, such as represented by the formula:



wherein M is as described; R<sub>22</sub> is methyl or hydrogen; n is a number especially 1 to about 10; m is 0 to about 10; and x is a number of 2 or more, e.g., usually sufficiently high to provide an average molecular weight of about 1,000 to about 1,000,000.

Another suitable stable metal-organic complex of a metal suitable for physical development with a polymer containing a ligand atom is a metal-organic complex of a metal suitable for physical development, especially silver, with a polymer containing thiaalkylacrylate units and/or thiaalkylmethacrylate units such as represented by the formula:



wherein M, R<sub>22</sub>, n, m and x are as described.

Examples of suitable metal-organic complexes according to the invention wherein the organic moiety is a described polymer include silver complexes with:

a terpolymer of (a) 3-thiapentylacrylate, (b) acrylic acid, and (c) 3-acryloxypropane-1-sulfonic acid sodium salt; a copolymer of (a) 3-thiapentylmethacrylate and (b) 3-acryloxypropane-1-sulfonic acid sodium salt; a terpolymer of (a) N-3-thiabutylacrylamide, (b) acrylamide, and (c) 2-methacryloxyethyl acetoacetate; and/or a copolymer of (a) S-2-methacryloxyethylisothiuronium methane-sulfonate and (b) 3-acryloxypropane-1-sulfonic acid sodium salt.

These polymers have a wide range of average molecular weight, but usually have an average molecular weight of about 100,000 or more.

The described polymers can be prepared employing methods of polymerization known in the art, e.g., such as methods set out in the described Schildknecht reference.

The invention includes other equivalent suitable sources of silver for physical development such as stable silver-organic complexes which are complexes of silver with:

1,10-phenanthroline



1(4-carboxyphenyl)-3,5-dimethyl-4-phenylpyrazole



Sodium dicyanamide



8-Hydroxyquinoline



8-hydroxyquinoline sulfate



saccharin



2,4-thiazolidinedione



Combinations of metal complexes can be employed according to the invention, such as combinations of silver complexes with gold, platinum or palladium complexes, or combinations of different organic complexing moieties, such as combinations of thiazoline thiones with alkynols or different thiazoline thiones with each other.

Metal and M as described herein with regard to metal-organic complexes refer to a metallic ion or the described metals in ionic form, such as a silver ion, mercury ion, platinum ion, gold ion, copper ion, and the like. In the described metal-organic complexes which are stable sources of metal for physical development according to the invention, it is believed the metal is in ionic form.

Whether a metal-organic complex employed according to the invention is suitably stable will depend on several factors,

such as the specific organic moiety, the components of the photographic element used, the affinity of the metal used for physical development, especially silver, to the organic moiety, the processing conditions and the like. Suitable stability is also related to keeping characteristics of a photographic element containing a described metal-organic complex. Usually, regarding this factor, compared to a control, if a photographic element does not show undesired loss in photographic speed and/or density after certain periods of time, such as after a few days, at about 50°C. and about 50 percent relative humidity, a metal-organic complex in the element is considered as suitably stable.

The elements described employing a silver-dye complex as a radiation-sensitive component, for example, with the described silver complexes as stable sources of silver for physical development can produce good reflection densities and high resolving power, e.g., resolving power over 2,000 line pairs per millimeter and many of the described elements have good stability, e.g., do not lose photographic speed or density after two weeks at about 50°C. and about 50 percent relative humidity.

Whether a metal-organic complex employed according to the invention is suitably stable depends heavily on the affinity for silver ion of the described organic moiety of the metal-organic complex used according to the invention. This can be measured as pAg. A suitable pAg range can vary.

A suitable pAg range in a radiation sensitive element according to the invention is about 2.0 to about 10 and a range of about 3 to about 7 is typically employed. If a pAg above about 10 is employed the risk of inhibition of desired development is great. But, if a pAg below about 2.0 is employed there is a risk of background fog formation. In the case of a photographic element containing a silver-dye complex as a radiation sensitive component, and a described silver-organic complex according to the invention as a stable source of silver for physical development, a concentration of about 0.01 mole to about 0.0001 mole of dye per mole of silver present and a concentration of about 0.2 mole to about 5.0 moles of organic moiety used to form the described silver-organic complexes of the invention per mole of silver in the element is suitable providing the desired pAg as described.

The concentration of described metal complexes suitable according to the invention can vary depending on the desired image, processing conditions, components of the photographic element, the affinity of the organic moiety of the described metal complexes for metal, especially silver, and the like, which can be determined by those skilled in the art. If the described silver complexes are incorporated in a photographic element containing a photographic silver salt, especially a described silver dye complex, a suitable ratio of (a) moles of organic moiety employed to form the desired silver complex as a stable source of silver for physical development to (b) moles of total silver in the photographic element is about 0.2 to about 7, depending upon the affinity of the organic moiety of the silver complex for silver. Especially suitable ratios of (a) moles of organic moiety employed to form the desired silver complex employed as a stable source for physical development to (b) moles of silver in an element containing the described silver complex are set out in the following examples. If the described silver complexes are employed in a processing composition, such as a physical developer composition, e.g., a physical developer solution with which a photographic element is contacted, higher concentrations of silver complex can be desirable, depending on the image desired, processing conditions and other factors described. A concentration of about 0.1 percent by weight to about 15 percent by weight of described metal complex of the total processing composition is usually suitable, but concentrations outside this range can be employed if desired.

While a wide range of ratios of concentration of described organic moiety to concentration of silver in a system according to the invention can be employed, a suitable concentration depends heavily on the affinity for silver ion of the described

organic moiety, which can be measured as pAg. Availability of silver ion can be measured using a pAg electrode. A low value indicates high silver ion activity or availability and vice versa.

The suitable concentration of total silver in coatings of photographic elements employing a silver-dye complex as a radiation-sensitive component and a described silver complex as a stable source of silver for physical development can vary over a wide range, but typically about 30 mg. per square foot to about 200 mg. per square foot of silver is suitable. It will be appreciated that this is a significantly higher concentration than employed in a coating containing only a silver-dye complex.

The described silver complexing agents of the invention, especially the described thiazoline-2-thiones and thiazolidine-2-thiones, can provide toning for the developed image.

The various layers of the photographic elements described herein can be hardened with any suitable hardener, including, for example, aldehyde hardeners, aziridine hardeners, hardeners which are derivatives of dioxane, oxypolysaccharides, such as oxystarch, oxy plant gums, and the like. The layers of the photographic element can contain hardeners such as alkali soluble bisulfite-aldehyde addition products which harden hydrophilic colloids such as gelatin at a pH greater than about 7. Such hardeners can conveniently be incorporated into photographic silver halide emulsion layers or other layers of an element particularly gelatin having layers, since such layers are generally coated under acid conditions, i.e., at a pH which is generally less than about 6. Suitable alkali metal bisulfitealdehyde addition products include, for example, sodium formaldehyde bisulfite, glutaraldehyde bis(sodium bisulfite), betamethyl glutaraldehyde bis(sodium bisulfite), maleic dialdehyde bis(sodium bisulfite), and the like.

Various colloids can be used alone or in combination as vehicles or binding agents in the photographic emulsions and elements employed in the practice of this invention. Among such materials are the natural and/or synthetic binding materials generally employed for this purpose including, for example, gelatin, colloidal albumin, water-soluble vinyl polymers as exemplified by mono- and polysaccharides, cellulose derivatives, proteins, water-soluble polyacrylamides, polyvinyl pyrrolidone, and the like. In addition to the hydrophilic colloids, the vehicle or binding agents can contain dispersed polymerized vinyl compounds particularly those which increase the dimensional stability of photographic materials. Suitable synthetic polymers of this type include water-insoluble polymers of alkyl acrylates and methacrylates, acrylic acid, sulfoalkyl acrylates or methacrylates and the like.

A wide range of photographic components can be employed as the described main photographic component used in a photographic element, composition and/or process of the invention. While some of the described stable metal-organic complexes used as a source of metal for physical development do have some photosensitivity they are used according to the invention as a source of metal for physical development and not as a radiation-sensitive component, i.e., a component which upon exposure to radiation forms latent image sites which can be physically developed. A preferred main photographic component is a silver-dye complex as described. If desired, silver halides can be employed in the photographic elements, processes and compositions of the invention, especially as the main photographic component, including any of the photographic silver halides as exemplified by silver bromide, silver iodide, silver chloride, mixed silver halides, such as silver chlorobromide, silver bromoiodide, and the like. The silver halides can be those which form latent images predominantly on the surface of the silver halide grains or those which form latent images inside the silver halide crystals, as exemplified by Davey and Knott, U.S. Pat. No. 2,592,250 issued Apr. 8, 1952, as well as direct positive emulsions, such as those described in Kendall and Hill, U.S. Pat. No. 2,541,472 issued Feb. 13, 1951. Other photographic silver salts can be employed, such as silver salts of sulfur-containing aliphatic

carboxylic acids, as described in U.S. Pat. No. 3,330,663 of Weyde et al. issued July 11, 1967.

The photographic layers described herein can be coated on a wide variety of supports. Typical flexible supports include those generally employed for photographic elements, such as cellulose nitrate film, cellulose acetate film, polyvinylacetal film, polystyrene film, polyethylene terephthalate film, and related films or resinous materials as well as glass, paper, metal and the like. Supports such as papers which are partially acetylated or coated with baryta or an olefin polymer, particularly a polymer of an alpha-olefin containing two to 10 carbon atoms as exemplified by polyethylene, polypropylene, ethylene-butene copolymers, and the like, give good results.

The photographic emulsions and elements of this invention can also contain additional addenda, particularly those known to be beneficial in photographic materials of this nature. For example, they can contain stabilizers or antifoggants such as cadmium, lead, mercury, gold, or other noble metal salts, spectral sensitizers, such as the cyanines, merocyanines, complex (trinuclear) cyanines, complex (trinuclear) merocyanines, styryls, hemicyanines, speed-increasing materials, such as polyalkylene glycols, onium salts and thioethers, plasticizers, coating aids such as anionic, nonionic and amphoteric surface active compounds, and the like. The photographic silver halide emulsions disclosed herein can also be chemically sensitized with compounds of the sulfur group, such as sulfur, selenium and tellurium sensitizers, noble metal salts, such as gold, or reduction sensitized with reducing agents or combinations of such materials. The photographic elements can contain fluorescent brighteners such as stilbenes, coumarins, benzothiazoles, benzoxazoles, imidazoles, etc. Suitable fluorescent brighteners are described in McFall et al. U.S. Pat. No. 2,933,390, British Patent 786,235, U.S. Pat. No. 3,025,242 and German Patent 1,150,274.

A wide range of coating methods can be employed for preparing photographic elements according to the invention. In general, any of those methods commonly employed in preparing coatings for photographic elements are suitable.

40 A silver halide developing agent can be employed in providing physical development according to the invention. A wide range of silver halide developing agents are suitable. These include polyhydroxybenzene developing agents, such as hydroquinone developing agents, e.g., hydroquinone, alkyl substituted hydroquinone, such as t-butyl hydroquinone, methyl hydroquinone, dimethyl hydroquinone, catechol, and pyrogallol, chloro-substituted hydroquinones, such as chlorohydroquinone, alkoxy-substituted hydroquinones, such as methoxy or ethoxy hydroquinone, aminophenol developing agents, such as N-methyl-p-aminophenol and 2,4-diaminophenols, ascorbic acid developing agents, pyrazolidone developing agents, including those described in British Patent 958,678 and British Patent 930,572, acyl derivatives of p-aminophenol, and the like. Such developing agents can be used alone or in combination. It is usually desirable that the developing agent employed be soluble in water. The suitable concentration can vary over wide ranges depending on the desired image, the components of the photographic element, processing conditions, and the like.

50 The desired silver complexes are suitable in layers of photographic elements used for color photography, such as emulsions containing color-forming couplers or emulsions developed by solutions containing couplers or other color-generating materials; emulsions of the mixed packet type, such as described in U.S. Pat. No. 2,698,794 of Godowsky issued July 9, 1955; or emulsions of the mixed grain type, such as described in U.S. Pat. No. 2,592,243 of Carroll and Hanson.

55 60 65 70 75 The described silver complexes as stable sources of silver for physical development can be employed in photographic elements processes and compositions intended for use in diffusion transfer processes which utilize undeveloped silver salts in the nonimage areas of the negative to form a positive by dissolving the undeveloped silver salts or complexes and

precipitating them on a receiving layer in close proximity to the original silver salt emulsion layer. Such processes are described, for example, in U.S. Pat. No. 3,020,155 to Yackel et al. issued Feb. 6, 1962, U.S. Pat. Nos. 2,584,029 issued Jan. 29, 1952; 2,698,236 issued Dec. 28, 1954; and 2,543,181 issued Feb. 27, 1951 of E. H. Land and U.S. Pat. No. 2,352,014 of Rott issued June 20, 1944. The invention can also be used in color transfer processes which utilize the diffusion transfer of developer, coupler or dye, from a light-sensitive layer to a second layer, such as described in U.S. Pat. No. 2,559,643 of Land, issued July 10, 1951; U.S. Pat. No. 2,698,798 issued Jan. 4, 1955; U.S. Pat. No. 2,756,142 of Yutzy issued July 14, 1956; U.S. Pat. No. 3,252,915 of Weyerts et al. issued May 31, 1966; and U.S. Pat. No. 3,227,550 of Whitman et al. issued Jan. 4, 1966. The described silver complexes are useful in other elements and processes designed for color photography, such as described in U.S. Pat. No. 3,242,294 of Barr et al. issued Mar. 29, 1966 and U.S. Pat. No. 2,252,718 of Mannes et al. issued Aug. 14, 1961.

The invention can be employed with photographic elements and processes designed for use in lithography, preparation of direct prints, or in colloid transfer processes, as well as in elements designed for processing in monobath processes, such as in monobath processes described in U.S. Pat. No. 2,875,048 of Haist et al. issued Feb. 24, 1959, and web-type processing such as described in U.S. Pat. No. 3,179,517 of Tregillus et al.

Another embodiment of the invention is a photographic process comprising physical development of a latent image in a radiation-sensitive metal salt employing a stable source of metal especially silver, for the described physical development which is a stable metal complex as described herein.

An especially suitable process, however, comprises physically developing a latent image in a photographic element containing (a) a silver-dye complex which has the property of forming active sites for physical development upon exposure to radiation and (b) a stable source of silver for physical development which is a stable metal complex, as described, wherein the metal is silver, with a silver halide developer solution.

A wide range of processing conditions can be employed depending on the desired image, photographic element processed, developer employed and the like. Processing is usually carried out under ambient conditions of temperature and pressure, e.g., a temperature of about 20° C. to about 30° C., but higher temperatures can be employed if desired, such as temperatures above about 50° C., e.g., about 50° to about 150° C.

The time required for processing can vary widely, such as from about 1 second to several minutes or more depending on processing conditions and desired image. Employing an element containing a described silver-dye complex and a described stable source of silver for physical development, a good image can be produced in about 2 to about 60 seconds when a silver halide developer solution is employed for processing.

Development activators which can be used according to the invention include any of those which provide the desired activation of the described developing agents. These include alkaline activators such as inorganic alkalis, for example, sodium hydroxide, potassium hydroxide and lithium hydroxide, alkali metal carbonates, such as sodium carbonate and potassium carbonate, and organic alkaline development activators such as quaternary ammonium bases and salts and similar alkaline materials and/or alkali releasing materials, and the like.

Processing compositions, such as developer solutions and/or stabilizer solutions and/or activator solutions, can be applied to or otherwise contacted with the described photographic elements in any suitable manner, including for instance, dipping, spraying and/or suitable surface applications, such as with rollers or other mechanical means.

A useful process according to the invention of effecting development of a photographic element containing a silver-dye complex, as described, and a silver-organic complex, as

described, which is a stable source of silver for physical development comprises contacting the photographic element with a silver halide developing agent in the presence of a development activator, such as contacting the photographic element with an aqueous alkaline developer solution. This silver halide developer can be a physical developer if desired, e.g., one containing a source of silver for physical development, such as a water-soluble silver salt, e.g., silver nitrate, and/or one of the described silver complexes.

A further embodiment of the invention is a photographic composition comprising (a) a stable source of metal for physical development which is a stable metal complex, as described herein, and (b) a silver-dye complex which has the property of forming active sites for physical development upon exposure to radiation. This photographic composition can be a photographic emulsion.

Another embodiment of the invention is a physical developer composition comprising:

- 20 A. a silver halide developing agent and/or other suitable reducing agent, and
- B. a stable source of metal for physical development which is a stable metal complex as described. This physical developer is typically an alkaline solution, such as an alkaline solution containing a polar solvent including, for example, water, ethylene glycol, alcohol, and the like.

It is often desirable to include a suitable hardener, as described herein, in the physical developer. A wide range of concentrations can be employed, depending on the element processed, processing conditions, components of the physical developer, and the like. A concentration of about 0.1 to about 1.5 percent by weight of hardener of the total physical developer composition is usually sufficient.

One or more components of the described physical developer can be stored in separate containers, such as in separate packets or bottles as part of a kit before use. At the time of or shortly before use, the component or components can be mixed together and/or diluted with a suitable solvent, such as water, to the desired concentration.

40 It can be advantageous in some cases to have an antifoggant present in a processing composition according to the invention and/or in the photographic element processed. Suitable antifoggants include organic antifoggants, such as benzotriazole, benzimidazole, 2-mercaptopbenzimidazole, and mercaptoazole antifoggants. An inorganic antifoggant, such as potassium bromide, potassium iodide and/or sodium bromide can be employed if desired. One of the advantages of the invention is that some of the organic complexing moieties can provide toning of the developed image. Some of the organic complexing moieties are also antifoggants.

The following examples are included for a further understanding of the invention.

#### EXAMPLE 1

A photographic element is prepared in Example 1 employing a coating of the following mixture on a film support:

|    | Component                                                                                                                       | Concentration<br>in milliliters |
|----|---------------------------------------------------------------------------------------------------------------------------------|---------------------------------|
| 60 | a. 0.002 molar aqueous solution of 1-carboxymethyl-5-[3-ethyl-2-benzoxazolinylidene]-ethylidene]-3-phenyl-2-thiohydantoin (dye) | 0.5                             |
| 65 | b. 0.2 molar aqueous solution of silver-p-toluenesulfonate                                                                      | 1.1                             |
| 70 | c. aqueous solution containing 10% by weight photographic gelatin                                                               | 5.5                             |
|    | d. aqueous solution containing 15% by weight saponin                                                                            | 0.25                            |
|    | e. aqueous solution containing 10% by weight formaldehyde                                                                       | 0.06                            |

One milliliter of solution of the organic moiety set out in following Table I on column A is added to the resulting mixture

before coating and the volume brought to about 12 ml. with water. This solution contains a concentration of described organic moiety sufficient to provide a preferred ratio of moles of organic moiety to moles of silver designated in column B thus forming the desired silver complex in situ. A plus sign (+) in column B indicates the useful range exceeds the designated value. The mixture is coated on a film support producing a coating containing 60 mg. of silver per square foot. After drying the element is exposed sensitometrically and the resulting latent image developed by immersing in the following solution:

|                   |         |
|-------------------|---------|
| Sodium sulfite    | 90.0 g. |
| Hydroquinone      | 45.0 g. |
| Sodium hydroxide  | 37.5 g. |
| Potassium bromide | 30.0 g. |
| Water to          | 1 l.    |

and fixed by immersing for 2 minutes in the following solution:

|                    |          |
|--------------------|----------|
| Sodium thiosulfate | 240.0 g. |
| Sodium sulfite     | 15.0 g.  |
| Acetic acid (28%)  | 48.0 cc. |
| Boric acid         | 7.5 g.   |
| Potassium alum     | 15.0 g.  |
| Water              | 1 l.     |

A high-resolution neutral image having high covering power (covering power=density/silver coverage in grams per square foot) and good reflection density is produced in each instance.

TABLE I

| Example | Column A:<br>moiety complexed<br>with silver as<br>stable source of<br>silver for physical<br>development | Column B:<br>ratio of moles<br>of organic<br>moiety to total<br>moles of silver<br>in coating | 35  | acid sodium salt) 1:1 or 1:3 mole<br>ratio                  |
|---------|-----------------------------------------------------------------------------------------------------------|-----------------------------------------------------------------------------------------------|-----|-------------------------------------------------------------|
| 1       | Mercaptoacetic acid                                                                                       | 0.35-0.50                                                                                     | 62  | 3-methyl-1-butyn-3-ol                                       |
| 2       | Mercaptopropionic acid                                                                                    | 0.25-0.35                                                                                     | 63  | 1,8 mole ethylene oxide adduct<br>of 3-methyl-1-butyn-3-ol  |
| 3       | Mercaptoisobutyric acid                                                                                   | 0.35-0.50                                                                                     | 64  | 5 mole ethylene oxide adduct<br>of 3-methyl-1-butyn-3-ol    |
| 4       | Mercaptosuccinic acid                                                                                     | 0.3-0.65                                                                                      | 65  | 3-methyl-1-pentyn-3-ol                                      |
| 5       | alpha-Mercaptoadipic acid                                                                                 | 0.5-0.7                                                                                       | 66  | 2.2 mole ethylene oxide adduct<br>of 3-methyl-1-pentyn-3-ol |
| 6       | L-cysteine                                                                                                | 0.2-0.5                                                                                       | 67  | 1-hexyn-3-ol                                                |
| 7       | Mercaptoacetanilide                                                                                       | 0.6-0.9                                                                                       | 68  | 1-ethynylcyclopentanol                                      |
| 8       | Thiobarbituric acid                                                                                       | 0.3-0.4                                                                                       | 69  | 1-ethynylcyclohexanol                                       |
| 9       | 1,3-diethyl-2-thiobarbituric<br>acid                                                                      | 1.5-3.0                                                                                       | 70  | 2.2 mole ethylene oxide adduct<br>of 1-ethynylcyclohexanol  |
| 10      | 2-Thiouracil                                                                                              | 0.5-0.7                                                                                       | 71  | 2-propynyl cyclohexylcarboxylate                            |
| 11      | Imidazolidine-2-thione                                                                                    | 0.6-0.9                                                                                       | 72  | 4-1-butyl-1-ethynylcyclohexanol                             |
| 12      | 1,3-bis(4-carboxyphenyl)-<br>1,3-dimethylthiourea                                                         | 0.8-1.2                                                                                       | 73  | 3-(diethylamino)-1-butyne                                   |
| 13      | 1,3-bis(2-carboxyethyl)-<br>benzimidazole-2-thione                                                        | 1.2-1.5                                                                                       | 74  | Methyl propiolate                                           |
| 14      | 1-(3,5-dicarboxyphenyl)-<br>5-mercaptotetrazole                                                           | 0.55-0.8                                                                                      | 75  | 3,5-dimethyl-1-hexyn-3-ol                                   |
| 15      | D-xylene diethyl mercaptal                                                                                | 1.2-2.0+                                                                                      | 76  | 4-(1-hydroxy-2-propynyl)<br>cyclohexene                     |
| 16      | 5,5'-diethiobis(1-phenyltetra-<br>zole)                                                                   | 0.6                                                                                           | 50  | 3-cyclopropyl-1-butyn-3-ol                                  |
| 17      | 4-carboxybenzyl dimethyl-<br>dithio-carbamate                                                             | 1.36                                                                                          | 77  | 3-phenyl-1-propyn-3-ol                                      |
| 18      | 11,14,17,20-tetrakis(hydroxymethyl)-<br>13,16,19-trioxa-4,7,10-trithia-<br>1,2,22-docosanetriol           | 1.8-2.0+                                                                                      | 78  | 3-(p-chlorophenyl)-1-butyn-3-ol                             |
| 19      | 2-hydroxyethylamino-oligoethylene-<br>sulfide                                                             | 0.6-0.8                                                                                       | 79  | 3-methyl-1-nonyn-3-ol, 10 mole<br>ethylene oxide adduct     |
| 20      | 4-(hydroxymethyl)cyclohexylmethyl-<br>amino oligoethylene sulfide                                         | 0.6-0.9                                                                                       | 80  | 1,10-phenanthroline                                         |
| 21      | 5-carboxy-2-phenyl-4-thiopyridine                                                                         | 4-0.7                                                                                         | 81  | 1-(4-carboxyphenyl)-3,5-dimethyl<br>4-phenylpyrazole        |
| 22      | 5-carbethoxy-1-methyl-2-phenyl-4-<br>thiopyrimidine                                                       | 1.0-1.3                                                                                       | 82  | Sodium dicyanamide ( $\text{Na}(\text{CN})_2$ )             |
| 23      | 5-methyloxazolidine-2-thione                                                                              | 0.6-0.7                                                                                       | 83  | 6-carboxy-7-hydroxy-1,3a,4-<br>triazaindene                 |
| 24      | 2-(carboxymethylthio)-5-phenyl-<br>1,3,4-oxadiazole                                                       | 1.0-3.0+                                                                                      | 84  | 8-hydroxyquinoline                                          |
| 25      | 4-(1,2-dicarboxyethylthio)-<br>5-phenylcatechol                                                           | 1.2-2.7                                                                                       | 85  | 8-hydroxyquinoline sulfate                                  |
| 26      | S-(o-carboxyphenyl)thioglycolic<br>acid                                                                   | 1.5-3.0+                                                                                      | 60  | Saccharin                                                   |
| 27      | 4-(methylthio)phenol                                                                                      | 4.0+                                                                                          | 86  | Pseudothiobutydantoin                                       |
| 28      | Phenylthioacetic acid                                                                                     | 1.0-3.0+                                                                                      | 87  | 2,4-thiazolidinedione                                       |
| 29      | 4-(carboxymethylthio)aniline                                                                              | 1.0-3.0                                                                                       | 88  | 5-sulfobenzotriazole                                        |
| 30      | 3-thiavaleric acid                                                                                        | 1.2-2.0+                                                                                      | 89  | (m-phenylenedioxy)diacetic acid                             |
| 31      | S-(carboxymethyl)isothiourea                                                                              | 0.8-2.1                                                                                       | 90  | Glycolic acid                                               |
| 32      | S-(2-carboxymethyl)isothiourea                                                                            | 0.2-2.0                                                                                       | 91  | Lactic acid                                                 |
|         |                                                                                                           |                                                                                               | 65  | Methylalactic acid                                          |
|         |                                                                                                           |                                                                                               | 92  | Malic acid                                                  |
|         |                                                                                                           |                                                                                               | 93  | Tartaric acid                                               |
|         |                                                                                                           |                                                                                               | 94  | Citric acid                                                 |
|         |                                                                                                           |                                                                                               | 95  | Tetrahydroxysuccinic acid                                   |
|         |                                                                                                           |                                                                                               | 96  | 12-hydroxystearic acid                                      |
|         |                                                                                                           |                                                                                               | 97  | Oxalic acid                                                 |
|         |                                                                                                           |                                                                                               | 98  |                                                             |
|         |                                                                                                           |                                                                                               | 99  |                                                             |
|         |                                                                                                           |                                                                                               | 100 |                                                             |

**EXAMPLE 101**

1.2-2.0+ 0.8-2.1 0.2-2.0 The procedure set out in Example 1 is repeated with a 75 silver-organic complex using organic moieties within the

scope of the following formula in place of the designated organic moiety of Examples 1-100:



wherein R<sub>30</sub>, R<sub>31</sub> and R<sub>32</sub> are set out respectively in column A, B and C of Table II. The concentration of described 4-thiazoline-2-thione is sufficient to provide a preferred ratio of moles of organic moiety to total moles of silver in the element. This is designated in column D of Table II. The resulting photographic element is exposed sensitometrically and the resulting latent image developed and fixed as set out in Example 1. A high-resolution neutral image having covering power and good reflection density is produced in each instance.

TABLE II

| Example | Column A, R <sub>30</sub>                         | n               | Column B, R <sub>31</sub>                                                       | Column C, R <sub>32</sub> | Column D |
|---------|---------------------------------------------------|-----------------|---------------------------------------------------------------------------------|---------------------------|----------|
| 101     | (CH <sub>2</sub> ) <sub>n</sub> COOH              | 1               | CH <sub>3</sub>                                                                 | H                         | 1.5-1.8  |
| 102     | (CH <sub>2</sub> ) <sub>n</sub> COOH              | 2               | CH <sub>3</sub>                                                                 | H                         | 1.6-2.0  |
| 103     | (CH <sub>2</sub> ) <sub>n</sub> COOH              | 3               | CH <sub>3</sub>                                                                 | H                         | 1.8-2.0  |
| 104     | (CH <sub>2</sub> ) <sub>n</sub> COOH              | 5               | CH <sub>3</sub>                                                                 | H                         | 1.8-2.0  |
| 105     | (CH <sub>2</sub> ) <sub>n</sub> COOH              | 1               | CH <sub>3</sub>                                                                 | COOH                      | 0.8-2.0  |
| 106     | (CH <sub>2</sub> ) <sub>n</sub> COOH              | 2               | CH <sub>3</sub>                                                                 | COOH                      | 1.5-2.0  |
| 107     | (CH <sub>2</sub> ) <sub>n</sub> COOH              | 3               | CH <sub>3</sub>                                                                 | COOH                      | 1.6-1.8  |
| 108     | (CH <sub>2</sub> ) <sub>n</sub> COOH              | 1               | CH <sub>3</sub>                                                                 | COOEt                     | 0.75-2.5 |
| 109     | (CH <sub>2</sub> ) <sub>n</sub> COOH              | 2               | CH <sub>3</sub>                                                                 | COOEt                     | 1.0-2.0  |
| 110     | (CH <sub>2</sub> ) <sub>n</sub> COOH              | 3               | CH <sub>3</sub>                                                                 | COOEt                     | 1.6-2.0  |
| 111     | (CH <sub>2</sub> ) <sub>n</sub> COOH              | 1               | CH <sub>3</sub> COOH                                                            | H                         | 1.0-2.0  |
| 112     | (CH <sub>2</sub> ) <sub>n</sub> COOH              | 3               | CH <sub>3</sub> COOH                                                            | H                         | 1.0-2.0  |
| 113     | (CH <sub>2</sub> ) <sub>n</sub> COOH              | 1               | CH <sub>3</sub>                                                                 | COOH <sub>3</sub>         | 0.9-1.4  |
| 114     | (CH <sub>2</sub> ) <sub>n</sub> COOH              | 2               | CH <sub>3</sub>                                                                 | COOH <sub>3</sub>         | 0.9-1.4  |
| 115     | (CH <sub>2</sub> ) <sub>n</sub> SO <sub>2</sub> H | 2               | CH <sub>3</sub>                                                                 | H                         | 0.4-1.4  |
| 116     | m-C <sub>6</sub> H <sub>4</sub> COOH              | CH <sub>3</sub> |                                                                                 | H                         | 0.9-1.4  |
| 117     | (CH <sub>2</sub> ) <sub>n</sub> COOH              | 1               | C <sub>6</sub> H <sub>5</sub>                                                   | H                         | 0.6-1.4  |
| 118     | CH <sub>3</sub> COOH                              | CH <sub>3</sub> |                                                                                 | H                         | 0.8-1.4  |
|         | CH <sub>3</sub>                                   |                 |                                                                                 |                           |          |
| 119     | Same as above                                     |                 | COOH                                                                            | H                         | 1.0-1.6  |
| 120     | do                                                |                 | COOEt                                                                           | H                         | 1.2-2.0  |
| 121     | do                                                |                 | CH <sub>3</sub> COOEt                                                           | H                         | 1.4-2.0  |
| 122     | (CH <sub>2</sub> ) <sub>n</sub> COOH              | 1               | CH <sub>3</sub> COOEt                                                           | H                         | 1.4-2.0  |
| 123     | (CH <sub>2</sub> ) <sub>n</sub> COOH              | 2               | CH <sub>3</sub> SO <sub>2</sub> (CH <sub>2</sub> ) <sub>3</sub> CH <sub>3</sub> | H                         | 0.8-1.4  |
| 124     | CH <sub>3</sub> COOH                              | CH <sub>3</sub> |                                                                                 | H                         | 1.0-2.0  |
|         | CH <sub>2</sub> COOH                              |                 |                                                                                 |                           |          |
| 125     | H                                                 |                 | COOH                                                                            | H                         | 0.1-0.4  |

## EXAMPLE 126

This illustrates a diffusion transfer process according to the invention.

A photographic element is prepared by coating the following mixture on a film support:

| Component                                                                                                                          | Milliliters |
|------------------------------------------------------------------------------------------------------------------------------------|-------------|
| a. aqueous solution containing 15% by weight of saponin                                                                            | 1.9         |
| b. 0.016 molar aqueous solution of 1-carboxymethyl-5-[1-(3-ethyl-2-benzoxazolinylidene)-ethylidene]-3-phenyl-2-thiohydantoin (dye) | 1.5         |
| c. 0.2 molar aqueous solution of silver-p-toluen sulfonate                                                                         | 28.0        |
| d. aqueous solution containing 15% by weight of photographic gelatin                                                               | 95.0        |
| e. 0.25 molar solution of 5-carboxy-3-(carboxymethyl)-4-methyl-4-thiazoline-2-thione (forms silver complex in situ)                |             |
| f. 7 N Sulfuric acid                                                                                                               | 28.0        |
| g. 0.16 molar aqueous ethanol solution of mucochloric acid                                                                         | 1.0         |
| h. 0.1 N aqueous sodium hydroxide solution                                                                                         | 7.5         |
|                                                                                                                                    | 4.5         |

This is coated on a film support at the rate of 60 mg. per square foot of silver. After drying, it is exposed sensitometrically. A paper receiver sheet containing colloidal silver development nuclei is soaked for 2 minutes in a monobath having the following composition:

2-methylaminoethanol (17.2% SO<sub>2</sub> adduct) 45 ml.  
Hydroquinone 11 g.

|                                  |        |
|----------------------------------|--------|
| Sodium thiosulfate pentahydrate  | 16 g.  |
| Sodium hydroxide                 | 15 g.  |
| 4-methyl-1-phenyl-3-pyrazolidone | 4.5 g. |

The paper receiver sheet is then laminated to the exposed coating for 30 seconds. A positive image is formed on the receiver sheet and has a clean background. The positive image has a maximum density of 1.2.

## EXAMPLE 127

This illustrates color processing according to the invention. A photographic element is prepared as set out in Example 101. After drying, the resulting coating is exposed sensitometrically. It is then immersed in a color developer containing a cyan coupler as described in U.S. Pat. No. 2,252,718 of Mannes et al. It is then immersed successively in a stop-fix

bath, a bleach bath, and a fix bath as described in this U.S. patent to provide the desired colored image. The resulting cyan image has good sharpness of detail over a range of densities.

Other color couplers which are suitable are set out in U.S. Pat. No. 3,113,864 of Yager et al.

## EXAMPLE 128

Good results are obtained when an element and process is employed according to U.S. Pat. No. 2,113,329 of Mannes issued Apr. 5, 1938 employing a silver complex of 5-carboxy-3-carboxymethyl-4-methyl-4-thiazolidone-2-thione as a stable source of silver for physical development, as set out in Example 1, in the initial development step of this color process.

## EXAMPLE 129

The procedure set out in the immediate preceding example is repeated employing 1-ethynylcyclopentanol in place of the described thiazoline-2-thione compound.

A good image is obtained.

## EXAMPLE 130

A good color image is obtained employing an element and process described in U.S. Pat. No. 2,304,940 of Mannes et al. using a photographic element containing incorporated described magenta couplers and cyan couplers with a green sensitive silver dye complex as described in French Patent 1,453,635 of Gilman, Goffe and Jones issued Aug. 16, 1966. A silver complex with 5-carboxy-3-carboxymethyl-4-methyl-4-thiazolidine-2-thione as a stable source of silver for physical development is employed as set out in Example 1, in this element designed for color processing.

## EXAMPLE 131

The procedure set out in the immediate preceding example is repeated employing 1-ethynylcyclopentanol in place of the described thiazoline-2-thione compound.

A good image is obtained.

## EXAMPLE 132

A good color image is also obtained employing an element and process described in U.S. Pat. No. 2,304,940 of Mannes et al. using a blue sensitive silver-dye complex and a yellow coupler in a first layer, a green sensitive silver-dye complex and a magenta coupler in a second layer and a red sensitive silver-dye complex and a cyan coupler in a third layer. The red sensitive silver-dye complex, green sensitive silver-dye complex and blue sensitive silver-dye complex are as described in French Patent 1,453,635 of Gilman, Goffe and Jones issued Aug. 16, 1966, and the described couplers are set out in Mees, "The Theory of the Photographic Process," Third Edition, (1966), page 394. A complex of silver with 5-carbethoxy-3-carboxymethyl-4-methyl-4-thiazolidine-2-thione is employed in each layer of the photographic element, as set out in Example 1, as a stable source of silver for physical development in the initial development step of the process.

The results of the preceding examples indicate that coatings are obtained designed for color processing which are less turbid than photographic silver halide coatings, provide high resolution and sharpness, provide advantageous spectral sensitivity, eliminate the necessity of a yellow filter layer to account for inherent blue sensitivity of silver halide and eliminate many complicated ripening holding, noodling and/or washing steps necessary in the preparation of photographic silver halide coatings.

## EXAMPLE 133

This is a comparative example illustrating certain advantages according to the invention.

Three photographic elements are prepared as in Example 1. Each one of the three, however, contains a different source of silver for physical development as follows:

- A. Silver-5-carbethoxy-3-carboxymethyl-4-methyl-4-thiazolidine-2-thione
- B. Silver thiosulfate (prior art)
- C. Silver-4,5-(2,3,D-fructopyrano)-2-oxazolidine-thione (prior art)

The coatings are exposed sensitometrically and developed as set out in Example 1. The following results are obtained:

| Coating | D <sub>max</sub>    | D <sub>min</sub> | Photographic Speed | Tone          |
|---------|---------------------|------------------|--------------------|---------------|
| A       | 2.1                 | 0.20             | 1.0                | Neutral Black |
| B       | brown fog, no image |                  |                    |               |
| C       | 1.4                 | 0.25             | 0.4-0.5            | Blue-gray     |

The results demonstrate that a combination of increased maximum density, better neutral black tone, and reduction of fog or stain, in addition to increased photographic speed can be obtained according to the invention as compared to use of related known sources of silver for physical development.

The elements, processes and compositions of the invention are useful in physical development of a latent image in an exposed radiation-sensitive titanium compound, such as titanium dioxide or a titanium dioxide dye complex, such as described in French Patent 1,437,765. Although the exact mechanism of reaction which takes place is not fully understood, it is believed that when a dye-sensitized titanium dioxide is employed with a described silver-dye complex in combination with a described silver-organic complex of the invention as a stable source of silver for physical development a bifunctional radiation-sensitive coating is provided. That is, two different types of radiation-sensitive compounds are provided which can be processed selectively to provide two dif-

ferent types of images. For example, employing a mixture of (a) silver-dye complex, as described herein, (b) a dye-sensitized titanium dioxide compound, as described in French Patent 1,437,765 and (c) a silver-organic complex, as described herein, as a stable source of silver for physical development, a radiation-sensitive element can be exposed with a high-intensity exposure. The resulting image is developed as described in Example 1 to provide only an image from the silver-dye complex. However, an exposure of about 10 to about 50 times less than the intense exposure followed by physical development after immersing in a solution containing a water-soluble silver salt, provides an image resulting from the titanium dioxide. This provides the advantage that a permanent silver image, which can be developed or not as desired, can be produced with the option of adding information later by means of the latent image in the titanium dioxide. Both the titanium dioxide and silver-dye complex, as described, provide sites for physical development using the stable sources of metal for physical development according to the invention.

## EXAMPLE 134

This illustrates the invention employing titanium dioxide, which is dye sensitized as a radiation-sensitive component.

A photographic element is prepared by mixing and coating the following components at 40° C. under red safe-light conditions:

| 30                                                                                                    | Component | Concentration |
|-------------------------------------------------------------------------------------------------------|-----------|---------------|
| a. 0.2 molar aqueous methanol solution of 5-carbethoxy-3-carboxymethyl-4-methyl-4-thiazoline-2-thione | 2 ml.     |               |
| b. 10% aqueous solution of photographic gelatin                                                       | 10 ml.    |               |
| c. 0.2 N aqueous solution of silver-p-toluene sulfonic acid                                           | 2 ml.     |               |
| d. suspension formed from:                                                                            | 6 ml.     |               |
| i. 6 g. titanium dioxide                                                                              |           |               |
| ii. 30 ml. water                                                                                      |           |               |
| iii. 12 mg. of a ligand dye, 1,2-dihydroxy-anthraquinone (alizarin) in 1 ml. dimethyl formamide,      |           |               |
| iv. 21 ml. of 10% aqueous solution of photographic grade gelatin                                      |           |               |
| e. 15% aqueous solution of saponin                                                                    | 0.4 ml.   |               |
| f. 10% aqueous solution of formaldehyde                                                               | 0.4 ml.   |               |

This composition is coated on a paper support at a rate of 50 0.009 inch wet thickness. The coating is dried and exposed sensitometrically using a 100-watt tungsten light source. The resulting coating is developed as set out in Example 1. Only an image characteristic of the exposed silver-dye complex is visible. After 80 minutes storage in the dark, the element is exposed sensitometrically a second time, for 10 seconds, on a portion of the element which contains no developed image. The element is then immersed in a 1 percent aqueous silver nitrate solution for 10 seconds followed by rinsing in water for 10 seconds and developing as set out in Example 1. A second image, of lower density than the silver-dye image and characteristic of a titanium dioxide sensitized with dye image, is developed.

The metal-organic complexes, described herein, can be employed in a physical development process as set out in U.S. Pat. No. 2,735,773 of Dippel and Houtman issued Feb. 21, 1956 or U.S. Pat. No. 2,764,484 of Jonge et al. issued Sept. 25, 1956. For example, according to the invention a radiation-sensitive material, such as a photographic element containing a silver-dye complex, subsequent to exposure is contacted in a suitable manner with mercurous ions, for example, in 0.01 N mercurous nitrate or a mercurous salt of one of the described compounds of the invention, and then is contacted in a suitable manner with a physical developer containing a metal-organic complex according to the invention, such as a silver-thiazoline-2-thione or silverthiazolidine-2-thione complex.

The described 2-furyl thioethers, especially 2-furyl thioethers which contain a carboxyalkylthio or carboxyarylkylthio group in the 2 position of a furan ring, can be prepared by a one step method by reacting (a) an aliphatic or aromatic mono- or dithiol with (b) a 2,5-diloweracyloxy-2,5-dihydrofuran; 2,5-dihydro-2,5-diloweralkoxyfuran; 2,5-dihydro-2,5-diloweralkoxy-2-methylfuran; or fumaric dialdehyde. This preparation is described in copending application Ser. No. 764,331 now U.S. Pat. No. 3,591,609, of R. A. Silverman filed concurrently herewith. For example (2-furylthio)-propionic acid can be prepared by refluxing thiopropionic acid with 2,5-dihydro-2,5-dimethoxyfuran in about stoichiometric concentrations in a suitable solvent such as acetonitrile or acetic acid.

The exact bonding in the reaction product of the described organic moieties and metal suitable for physical development as described, is not fully understood. These reaction products, such as the reaction product of a thiazoline-2-thione compound with a water-soluble silver salt, such as silver nitrate, are designated as metal-organic complexes. These can include bonding which is covalent, ionic, or some other type. For example, a described metal-organic complex can be a so-called metal-organic salt, e.g., a silver salt, containing bonding which is characteristic of metal salts.

The invention has been described in detail with particular reference to preferred embodiments thereof, but it will be understood that variations and modifications can be effected within the spirit and scope of the invention as described hereinabove and as defined in the appended claims.

I claim:

1. A photographic element comprising a support, a radiation-sensitive silver-dye complex which has the property of forming active sites for physical development upon exposure to radiation and a stable source of metal for physical development which is a stable metal-organic complex of a metal suitable for physical development with a compound which is: a thiazoline thione, a thiazolidine thione, a thiopyrimidine, a dithiocarbamate represented by the formula:



a thiourea derivative represented by the formula:



a pseudothiohydantoin represented by the formula:



a imidazolidine, an imidazoline, an isothiourea derivative represented by the formula:



a mercaptocarboxylic acid, a mercaptoacetyl amide, an alkyne compound represented by the formula:



a hydroxyalkyl carboxylic acid, a hydroxy heterocyclic carboxylic acid, a thiaalkyl compound represented by the formula:



a dithiaalkyl compound represented by the formula: [(X-



an oligothiaalkyl compound represented by the formula:



5 oxalic acid, a phenylene dioxy dialkyl carboxylic acid, succinic acid, or a polymer containing a ligand atom having the property of complexing a metal suitable for physical development, wherein R<sub>1</sub>, R<sub>2</sub>, R<sub>4</sub> and R<sub>5</sub> are hydrogen, alkyl containing one to 20 carbon atoms, acyl containing one to five carbon atoms, aryl containing six to 30 carbon atoms, or atoms completing a five- or six-member heterocyclic ring; R<sub>15</sub> is hydrogen, aryl containing six to 30 carbon atoms, alkyl containing one to 20 carbon atoms, or atoms completing a ring with R<sub>16</sub>; R<sub>16</sub> is hydrogen, aryl containing six to 30 carbon atoms, alkyl containing one to 20 carbon atoms, or atoms completing a ring with R<sub>17</sub>; R<sub>17</sub> is —P—R<sub>18</sub>, —S—R<sub>19</sub>.



20 or an alkylene oxide polymer adduct or atoms completing a ring with R<sub>16</sub> wherein R<sub>18</sub>, R<sub>19</sub>, R<sub>20</sub> and R<sub>21</sub> are each hydrogen, acyl containing one to five carbon atoms, or alkyl containing one to 20 carbon atoms; wherein Z or X is a five- or six-member heterocyclic ring, aryl containing six to 30 carbon atoms, alkyl containing one to 20 carbon atoms, or acyl containing one to five carbon atoms; Z' is Z or hydrogen; Y is alkylene containing one to five carbon atoms; n is 1 to 10.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185



a thiourea derivative represented by the formula: [(VI)]



a pseudothiohydantoin represented by the formula: [(VIII)]



an imidazolidine, an imidazoline, an isothiourea derivative represented by the formula: [(XI)]



a mercaptocarboxylic acid, a mercaptoacetyl amide, an alkyne compound represented by the formula: [(XIV)]



a hydroxyalkyl carboxylic acid, hydroxy heterocyclic carboxylic acid, a thiaalkyl compound represented by the formula:



a dithiaalkyl compound represented by the formula:



an oligothiaalkyl compound represented by the formula:



oxalic acid, a phenylene dioxy dialkyl carboxylic acid, succinic acid, or a polymer containing a ligand atom having the property of complexing a metal suitable for physical development, wherein R<sub>1</sub>, R<sub>2</sub>, R<sub>4</sub> and R<sub>5</sub> are hydrogen, alkyl containing one to 20 carbon atoms, acyl containing one to five carbon atoms, aryl containing six to 30 carbon atoms, or atoms completing a five- or six-member heterocyclic ring; R<sub>15</sub> is hydrogen, aryl containing six to 30 carbon atoms, alkyl containing one to 20 carbon atoms, or atoms completing a ring with R<sub>16</sub>; R<sub>16</sub> is hydrogen, aryl containing six to 30 carbon atoms, alkyl containing one to 20 carbon atoms, or atoms completing a ring with R<sub>16</sub>; R<sub>16</sub> is hydrogen, aryl containing six to 30 carbon atoms, alkyl containing one to 20 carbon atoms, or atoms completing a ring with R<sub>17</sub>; R<sub>17</sub> is —O—R<sub>18</sub>, —S—R<sub>19</sub>,



or an alkylene oxide polymer adduct or atoms completing a ring with R<sub>16</sub>, wherein R<sub>18</sub>, R<sub>19</sub>, R<sub>20</sub>, and R<sub>21</sub> are each hydrogen, acyl containing one to five carbon atoms, or alkyl containing one to 20 carbon atoms; wherein Z or Z' is a five- or six-member heterocyclic ring, aryl containing six to 30 carbon atoms, alkyl containing one to 20 carbon atoms, or acyl containing one to five carbon atoms; Z' is Z or hydrogen; Y is alkylene containing one to five carbon atoms; n is 1 to 10.

13. A photographic process as in claim 12 comprising physical development of a latent image in an element which contains a layer sensitive to the red region of the spectrum, a layer sensitive to the green region of the spectrum, and a layer sensitive to the blue region of the spectrum.

14. A photographic process as in claim 12 wherein said metal is silver and said metal complex is a silver complex.

15. The process of claim 14 wherein the photographic process is a diffusion transfer process.

16. A photographic composition comprising a radiation-sensitive silver-dye complex and a stable source of metal for physical development of a latent image in said silver-dye complex, said stable source of metal being a stable metal-organic complex of a metal suitable for physical development with a compound which is:

a thiazoline thione, a thiazolidine thione, a thiopyrimidine, a dithiocarbamate represented by the formula: [(V)]



a thiourea derivative represented by the formula:



a pseudothiohydantoin represented by the formula: [(VIII)]



an imidazolidine, an imidazoline, an isothiourea derivative represented by the formula: [(XI)]



a mercaptocarboxylic acid, mercaptoacetyl amide, an alkyne compound represented by the formula: [(XIV)]



a hydroxyalkyl carboxylic acid, a hydroxy heterocyclic carboxylic acid, a thiaalkyl compound represented by the formula:



a dithiaalkyl compound represented by the formula:



an oligothiaalkyl compound represented by the formula:



oxalic acid, a phenylene dioxy dialkyl carboxylic acid, succinic acid, or a polymer containing a ligand atom having the property of complexing a metal suitable for physical development, wherein R<sub>1</sub>, R<sub>2</sub>, R<sub>4</sub> and R<sub>5</sub> are hydrogen, alkyl containing one to 20 carbon atoms, acyl containing one to five carbon atoms, aryl containing six to 30 carbon atoms, or atoms completing a five- or six-member heterocyclic ring; R<sub>15</sub> is hydrogen, aryl containing six to 30 carbon atoms, alkyl containing one to 20 carbon atoms, or atoms completing a ring with R<sub>16</sub>; R<sub>16</sub> is hydrogen, aryl containing six to 30 carbon atoms, alkyl containing one to 20 carbon atoms, or atoms completing a ring with R<sub>17</sub>; R<sub>17</sub> is —O—R<sub>18</sub>, —S—R<sub>19</sub>,

completing a ring with  $R_{17}$ ;  $R_{17}$  is  $-\text{O}-R_{18}$ ,  $-\text{S}-R_{19}$ ,



5

or an alkylene oxide polymer adduct or atoms completing a ring with  $R_{16}$  wherein  $R_{18}$ ,  $R_{19}$ ,  $R_{20}$  and  $R_{21}$  are each hydrogen, acyl containing one to five carbon atoms, or alkyl containing one to 20 carbon atoms; wherein  $Z$  or  $X$  is a five- or six-member heterocyclic ring, aryl containing six to 30 carbon atoms, alkyl containing one to 20 carbon atoms, or acyl containing one to five carbon atoms;  $Z'$  is  $Z$  or hydrogen,  $Y$  is alkylene containing one to five carbon atoms;  $n$  is 1 to 10.

10

17. A photographic composition as in claim 16 wherein said metal-organic complex is a silver complex.

15

18. A photographic composition as in claim 16 wherein said metal-organic complex is a complex of silver with a 4-thiazoline-2-thione.

20

19. A photographic composition as in claim 16 wherein said metal is silver and said composition has a pAg range of about 2.0 to about 10.

25

20 A photographic composition as in claim 16 which additionally contains a photographic silver halide.

30

21. A physical developer composition comprising (a) a silver halide developing agent, and (b) a stable source of metal for physical development which is a stable metal organic complex of metal suitable for physical development with a compound which is:

a thiazoline thione, a thiazolidine thione, a thiopyrimidine, a dithiocarbamate represented by the formula: [(V)]



35

a thiourea derivative represented by the formula: [(VI)]



40

a pseudothiohydantoin represented by the formula: [(VIII)]



50

45 or an alkylene oxide polymer adduct or atoms completing a ring with  $R_{16}$  wherein  $R_{18}$ ,  $R_{19}$ ,  $R_{20}$  and  $R_{21}$  are each hydrogen, acyl containing one to five carbon atoms, or alkyl containing one to 20 carbon atoms; wherein  $Z$  or  $X$  is a five- or six-member heterocyclic ring, aryl containing six to 30 carbon atoms, alkyl containing one to 20 carbon atoms, or acyl containing one to five carbon atoms;  $Z'$  is  $Z$  or hydrogen;  $Y$  is alkylene containing one to five carbon atoms;  $n$  is 1 to 10.

50 22. The physical developer composition of claim 21 wherein the composition is an alkaline solution.

23. A physical developer composition as in claim 21 wherein said metal complex is a silver complex.

55 \* \* \* \* \*

60

65

70

75

an imidazolidine, an imidazoline, an isothiourea derivative represented by the formula: [(XI)]



a mercaptocarboxylic acid, a mercaptoacetyl amide, an alkyne compound represented by the formula: [(XIV)]



a hydroxylcarboxylic acid, a hydroxy heterocyclic carboxylic acid, a thiaalkyl compound represented by the formula:

[(XVI)] X — S — Z

a dithiaalkyl compound represented by the formula:

[(XVII)] X — S — S — Z

an oligothiaalkyl compound represented by the formula:

[(XVIII)] X — S — Y — S —  $n$  Z' oxalic acid, a phenoxy diacyl carboxylic acid, succinic acid, or a polymer containing a ligand atom having the property of complexing a metal suitable for physical development, wherein  $R_1$ ,  $R_2$ ,  $R_4$  and  $R_5$  are hydrogen, alkyl containing one to 20 carbon atoms, acyl containing one to five carbon atoms, aryl containing six to 30 carbon atoms, or atoms completing a five- or six-member heterocyclic ring;  $R_{15}$  is hydrogen, aryl containing six to 30 carbon atoms, alkyl containing one to 20 carbon atoms, or atoms completing a ring with  $R_{16}$ ;  $R_{16}$  is hydrogen, aryl containing six to 30 carbon atoms, alkyl containing one to 20 carbon atoms, or atoms completing a ring with  $R_{17}$ ,  $R_{17}$  is  $-\text{O}-R_{18}$ ,  $-\text{S}-R_{19}$ ,



55 or an alkylene oxide polymer adduct or atoms completing a ring with  $R_{16}$  wherein  $R_{18}$ ,  $R_{19}$ ,  $R_{20}$  and  $R_{21}$  are each hydrogen, acyl containing one to five carbon atoms, or alkyl containing one to 20 carbon atoms; wherein  $Z$  or  $X$  is a five- or six-member heterocyclic ring, aryl containing six to 30 carbon atoms, alkyl containing one to 20 carbon atoms, or acyl containing one to five carbon atoms;  $Z'$  is  $Z$  or hydrogen;  $Y$  is alkylene containing one to five carbon atoms;  $n$  is 1 to 10.

22. The physical developer composition of claim 21 wherein the composition is an alkaline solution.

23. A physical developer composition as in claim 21 wherein said metal complex is a silver complex.